

## UNITED STATES PATENT OFFICE

LOGAN A. DILS, OF CHICAGO, ILLINOIS, ASSIGNOR TO KELLOGG DILS, INC., OF CHICAGO, ILLINOIS, A CORPORATION OF DELAWARE

## METHOD OF TREATING FIBERS FOR PAPER MAKING AND OTHER USES

No Drawing. Application filed July 24, 1930, Serial No. 470,536. Renewed December 12, 1931.

This invention relates to a process of treating certain classes of woody fibers, such as hemp, flax straw, bagasse, and the like, for the purpose of freeing the cellulose fibers thereof from the enveloping lignin in order to obtain the said fibers for paper making and other uses. With this object in view the invention consists, generally stated, in subjecting the said woody materials to the action of an aqueous solution of sodium borate, sodium hydroxide and trisodium phosphate at atmospheric pressure, for a period of time varying from ten to twenty minutes, depending upon the specific woody material under treatment, at a temperature of approximately 220° F. to 225° F., and then taking the cooked woody materials and subjecting them to the action of a beater for a period varying from one to three hours. When bagasse is thus "cooked" in a solution for a period varying from ten to fifteen minutes, and then subjected to the action of a beater for a period varying from one to three hours, the fibers are found to be of most excellent quality for certain classes of papers, such as a substitute for manila paper and cover stock.

The specific proportions of the chemicals employed may vary somewhat, but it has been found that the following formula gives most excellent results, that is, a solution composed of:

|                      | Per cent |
|----------------------|----------|
| Water                | 50       |
| Sodium borate        | 39       |
| Sodium hydroxide     | 10       |
| Tri-sodium phosphate | 1        |

The chemicals are first preferably mixed together until they begin to liquefy or assume the form of a thick heavy paste. This mixture of chemicals is then placed in an open vessel and the water added and the temperature brought up to approximately 220° F. by the application of extraneous heat, such, for example, as by the use of a gas burner.

The woody material, such as hemp, flax straw, bagasse or the like, is then subjected to the action of this solution for a period of approximately twelve minutes. The period of time may be slightly less or slightly more

than this, depending somewhat upon the class of the material being treated, or "cooked", as it is technically known.

After the woody material has thus been acted upon by said chemical solution, it is taken therefrom and placed in an ordinary beater of the kind usually employed in paper making plants. If old hemp rope forms the starting woody material, it should be beaten for from fifteen to twenty minutes. With bagasse it has been found that beating for a period of one hour gives very satisfactory results as does beating for two or three hours.

By this process fibrous woody materials of the character indicated can be "cooked" at atmospheric pressure, within a period of about fifteen minutes, and then beaten, and is ready for use in paper making within an hour or two additional, and fibers of a very superior quality for use in paper making or other uses obtained.

What is claimed is:

1. The method of treating woody materials, which consists in subjecting the same to the action of an aqueous solution of sodium borate, sodium hydroxide and tri-sodium phosphate.
2. The method of treating woody materials, which consists in subjecting the same to the action of an aqueous solution of sodium borate, sodium hydroxide and tri-sodium phosphate at atmospheric pressure.

3. The method of treating woody materials, which consists in subjecting the same to the action of an aqueous solution of sodium borate, sodium hydroxide and tri-sodium phosphate at atmospheric pressure for a period of approximately 12 minutes.

4. The method of treating woody materials, which consists in subjecting the same to the action of an aqueous solution of sodium borate, sodium hydroxide and tri-sodium phosphate at a temperature of approximately 220° F.

5. The method of treating woody materials, which consists in subjecting the same to the action of an aqueous solution of sodium borate, sodium hydroxide and tri-sodium phosphate at atmospheric pressure

and at a temperature of approximately 220° F.

6. The method of treating woody materials, which consists in subjecting the same to the action of an aqueous solution of sodium borate, sodium hydroxide and tri-sodium phosphate for a period of approximately 12 minutes.

10 7. The method of treating woody materials, which consists in subjecting the same to the action of an aqueous solution of sodium borate, sodium hydroxide and tri-sodium phosphate at atmospheric pressure for a period of approximately 12 minutes and at a temperature of about 220° F.

8. The method of treating woody materials, which consists in subjecting the same to the action of an aqueous solution of sodium borate, sodium hydroxide and tri-sodium phosphate and then removing the woody material from said solution and beating the same.

9. The method of treating woody materials, which consists in subjecting the same to the action of an aqueous solution of sodium borate, sodium hydroxide and tri-sodium phosphate at atmospheric pressure and then removing the woody material from the solution and beating the same.

30 10. The method of treating woody materials, which consists in subjecting the same to the action of an aqueous solution of sodium borate, sodium hydroxide and tri-sodium phosphate at atmospheric pressure for a period of approximately 12 minutes and then removing the woody material from the solution and beating the same.

35

11. The method of treating woody materials, which consists in subjecting the same to the action of an aqueous solution of sodium borate, sodium hydroxide and tri-sodium phosphate at a temperature of approximately 220° F. and then removing the woody material from the solution and beating the same.

45 12. The method of treating woody ma-  
terials, which consists in subjecting the same  
to the action of an aqueous solution of sodium  
borate, sodium hydroxide and tri-sodium  
phosphate at atmospheric pressure and at a  
50 temperature of approximately 220° F. and  
then removing the woody material from the  
solution and beating the same.

13. The method of treating woody materials, which consists in subjecting the same to the action of an aqueous solution of sodium borate, sodium hydroxide and tri-sodium phosphate for a period of approximately 12 minutes and then removing the woody material from the solution and beating the same.

14. The method of treating woody materials, which consists in subjecting the same to the action of an aqueous solution of sodium borate, sodium hydroxide and tri-sodium phosphate at atmospheric pressure for a period of approximately 12 minutes and at

a temperature of about 220° F. and then removing the woody material from the solution and beating the same.

15. The method of treating woody materials, which consists in subjecting the same to the action of an aqueous solution of sodium borate, sodium hydroxide and tri-sodium phosphate and then removing the woody material from said solution and beating the same for from one to two hours.

16. The method of treating woody materials, which consists in subjecting the same to the action of an aqueous solution of sodium borate, sodium hydroxide and tri-sodium phosphate at atmospheric pressure and then removing the woody material from the solution and beating the same for from one to two hours. 80

17. The method of treating woody materials, which consists in subjecting the same to the action of an aqueous solution of sodium borate, sodium hydroxide and tri-sodium phosphate at atmospheric pressure for a period of approximately 12 minutes and then removing the woody material from the solution and beating the same for from one to two hours. 85 90

18. The method of treating woody materials, which consists in subjecting the same to the action of an aqueous solution of sodium borate, sodium hydroxide and tri-sodium phosphate at a temperature of approximately 220° F. and then removing the woody material from the solution and beating the same for from one to two hours. 95

19. The method of treating woody materials, which consists in subjecting the same to the action of an aqueous solution of sodium borate, sodium hydroxide and tri-sodium phosphate at atmospheric pressure and at a temperature of approximately 220° F. and then removing the woody material from the solution and beating the same for from one to two hours.

20. The method of treating woody materials, which consists in subjecting the same to the action of an aqueous solution of sodium borate, sodium hydroxide and tri-sodium phosphate for a period of approximately 12 minutes and then removing the woody material from the solution and beating the same for from one to two hours. 110  
115

21. The method of treating woody materials, which consists in subjecting the same to the action of an aqueous solution of sodium borate, sodium hydroxide and tri-sodium phosphate at atmospheric pressure for a period of approximately 12 minutes and at a temperature of about 220° F. and then removing the woody material from the solution and beating the same for from one to two hours.

22. The method of treating woody materials, which consists in subjecting the same to a solution comprising approximately 50. 130

- percent water, 39. percent sodium borate, 10. percent sodium hydroxide, and 1. percent tri-sodium phosphate.
23. The method of treating woody materials, which consists in subjecting the same to a solution comprising approximately 50. percent water, 39. percent sodium borate, 10. percent sodium hydroxide, and 1. percent tri-sodium phosphate, at atmospheric pressure.
- 10 24. The method of treating woody materials, which consists in subjecting the same to a solution comprising approximately 50. percent water, 39. percent sodium borate, 10. percent sodium hydroxide, and 1. percent tri-sodium phosphate for a period of approximately 12 minutes.
- 20 25. The method of treating woody materials, which consists in subjecting the same to a solution comprising approximately 50. percent water, 39. percent sodium borate, 10. percent sodium hydroxide, and 1. percent tri-sodium phosphate, at a temperature of about 220° F.
- 25 26. The method of treating woody materials, which consists in subjecting the same to a solution comprising approximately 50. percent water, 39. percent sodium borate, 10. percent sodium hydroxide, and 1. percent tri-sodium phosphate at atmospheric pressure, for a period of approximately 12 minutes.
- 30 27. The method of treating woody materials, which consist in subjecting the same to a solution comprising approximately 50. percent water, 39. percent sodium borate, 10. percent sodium hydroxide, and 1. percent tri-sodium phosphate at atmospheric pressure at a temperature of about 220° F.
- 0 28. The method of treating woody materials, which consists in subjecting the same to a solution comprising approximately 50. percent water, 39. percent sodium borate, 10. percent sodium hydroxide, and 1. percent tri-sodium phosphate, at atmospheric pressure for a period of approximately 12 minutes and at a temperature of about 220° F.
- 5 29. The method of treating woody materials, which consists in subjecting the same to a solution comprising approximately 50. percent water, 39. percent sodium borate, 10. percent sodium hydroxide, and 1. percent tri-sodium phosphate, and then beating the same.
- 10 30. The method of treating woody materials, which consists in subjecting the same to a solution comprising approximately 50. percent water, 39. percent sodium borate, 10. percent sodium hydroxide, and 1. percent tri-sodium phosphate at atmospheric pressure, and then beating the same.
- 15 31. The method of treating woody materials, which consists in subjecting the same to a solution comprising approximately 50. percent water, 39. percent sodium borate, 10. percent sodium hydroxide, and 1. percent tri-sodium phosphate for a period of approximately 12 minutes, and then beating the same.
32. The method of treating woody materials, which consists in subjecting the same to a solution comprising approximately 50. percent water, 39. percent sodium borate, 10. percent sodium hydroxide, and 1. percent tri-sodium phosphate, at a temperature of about 220° F., and then beating the same.
- 75 33. The method of treating woody materials, which consists in subjecting the same to a solution comprising approximately 50. percent water, 39. percent sodium borate, 10. percent sodium hydroxide, and 1. percent tri-sodium phosphate at atmospheric pressure, for a period of approximately 12 minutes, and then beating the same.
- 80 34. The method of treating woody materials, which consists in subjecting the same to a solution comprising approximately 50. percent water, 39. percent sodium borate, 10. percent sodium hydroxide, and 1. percent tri-sodium phosphate at atmospheric pressure at a temperature of about 220° F., and then beating the same.
- 85 35. The method of treating woody materials, which consists in subjecting the same to a solution comprising approximately 50. percent water, 39. percent sodium borate, 10. percent sodium hydroxide, and 1. percent tri-sodium phosphate, at atmospheric pressure for a period of approximately 12 minutes and at a temperature of about 220° F., and then beating the same.
- 90 36. The process of treating bagasse, which consists in subjecting the same to an aqueous solution of sodium borate, sodium hydroxide and tri-sodium phosphate.
- 95 37. The process of treating bagasse, which consists in subjecting the same to an aqueous solution of sodium borate, sodium hydroxide and tri-sodium phosphate, at atmospheric pressure.
- 100 38. The process of treating bagasse, which consists in subjecting the same to an aqueous solution of sodium borate, sodium hydroxide and tri-sodium phosphate, for approximately 12 minutes.
- 105 39. The process of treating bagasse, which consists in subjecting the same to an aqueous solution of sodium borate, sodium hydroxide and tri-sodium phosphate, at a temperature of about 220° F.
- 110 40. The process of treating bagasse, which consists in subjecting the same to an aqueous solution of sodium borate, sodium hydroxide and tri-sodium phosphate, at atmospheric pressure, for approximately 12 minutes.
- 115 41. The process of treating bagasse, which consists in subjecting the same to an aqueous solution of sodium borate, sodium hydroxide and tri-sodium phosphate, at atmospheric pressure, at a temperature of about 220° F.
- 120 42. The process of treating bagasse, which consists in subjecting the same to an aqueous solution of sodium borate, sodium hydroxide and tri-sodium phosphate, for approximate-
- 125 130

ly 12 minutes, and at a temperature of about 220° F.

43. The process of treating bagasse, which consists in subjecting the same to an aqueous 5 solution of sodium borate, sodium hydroxide and tri-sodium phosphate, and then beating the same.

44. The process of treating bagasse, which consists in subjecting the same to an aqueous 10 solution of sodium borate, sodium hydroxide and tri-sodium phosphate, at atmospheric pressure, and then beating the same.

45. The process of treating bagasse, which consists in subjecting the same to an aqueous 15 solution of sodium borate, sodium hydroxide and tri-sodium phosphate, for approximately 12 minutes, and then beating the same.

46. The process of treating bagasse, which consists in subjecting the same to an aqueous 20 solution of sodium borate, sodium hydroxide and tri-sodium phosphate, at a temperature of about 220° F., and then beating the same.

47. The process of treating bagasse, which consists in subjecting the same to an aqueous 25 solution of sodium borate, sodium hydroxide and tri-sodium phosphate, at atmospheric pressure, for approximately 12 minutes, and then beating the same.

48. The process of treating bagasse, which 30 consists in subjecting the same to an aqueous solution of sodium borate, sodium hydroxide, and tri-sodium phosphate, at atmospheric pressure, at a temperature of about 220° F., and then beating the same.

49. The process of treating bagasse, which 35 consists in subjecting the same to an aqueous solution of sodium borate, sodium hydroxide and tri-sodium phosphate, for approximately 12 minutes, and at a temperature of about 220° F., and then beating the same.

50. The process of treating bagasse which 40 consists in subjecting the same for about 12 minutes to the action of a solution comprising approximately the following proportions: Water 50%; sodium borate 39%; sodium hydroxide 10%; and tri-sodium phosphate 1%, at a temperature of about 220° F.

51. The process of treating bagasse which 45 consists in subjecting the same for about 12 minutes to the action of a solution comprising approximately the following proportions: Water 50%; sodium borate 39%; sodium hydroxide 10%; and tri-sodium phosphate 1%, at a temperature of about 220° F., and then beating the bagasse for 55 from one to three hours.

In testimony whereof I have signed this specification.

60 LOGAN A. DILS.